

June 7, 1949.

H. BIENFAIT ET AL

2,472,189

THERMIONIC TUBE HAVING A SECONDARY-EMISSION ELECTRODE

Filed March 22, 1943



FIG. 1



FIG. 2

CORNELIS FREDERIK VEENEMANS  
• HENRI BIENFAIT  
INVENTORS

BY   
ATTORNEY

## UNITED STATES PATENT OFFICE

2,472,189

## THERMIONIC TUBE HAVING A SECONDARY-EMISSION ELECTRODE

Henri Bienfait and Cornelis Frederik Veenemans,  
Eindhoven, Netherlands, assignors to Hartford  
National Bank and Trust Company, Hartford,  
Conn., as trustee

Application March 22, 1943, Serial No. 480,102  
In the Netherlands July 3, 1941

Section 1, Public Law 690, August 8, 1946  
Patent expires July 3, 1961

2 Claims. (Cl. 250—174)

1

This invention relates to thermionic tubes provided with a secondary-emission electrode and more particularly to such tubes in which the secondary emission is brought about by an active layer consisting of caesium oxide, which is applied to the secondary-emission electrode.

Thermionic tubes containing a secondary-emission electrode covered with caesium oxide as an active material are already known.

Further, it is already known to cool secondary-emission electrodes; to this end, it has been suggested either to connect cooling bodies to the secondary-emission electrodes, or to cool the latter with the aid of a running liquid.

Furthermore, in thermionic tubes it was already general practice to cover definite electrodes with a black substance in order to improve the radiation of heat and thus maintain the temperature of the electrode concerned at a low value. The black material used is frequently carbon.

In the accompanying drawing Figure 1 shows the steps of the method according to the invention and Figure 2 shows an enlarged cross-section of a portion of an electrode made in accordance with the invention.

In Figure 1 the rectangles represent the successive steps of the method of the invention. The finished electrode shown in Figure 2 comprises a base on which heat-radiating black metal particles are disposed and about which particles emissive material is deposited.

It has been found, however, that carbon is not adapted to be applied to parts of secondary-emission electrodes which contain caesium oxide as active material, since carbon very easily absorbs or adsorbs caesium. Since the active caesium coating is almost solely obtained by applying caesium to the secondary-emission electrode by vaporisation and subsequently oxidising, good dosing of the caesium is impossible if part of the electrode is covered with carbon. On the other hand, it is desirable that on the secondary-emission electrode or in the vicinity thereof there be a material capable of binding small quantities of caesium.

Also the cooling of the secondary-emission electrode is desirable, since the heating of the electrode produced during operation injuriously affects the emission. The temperature of the

secondary-emission electrode during operation must in general not exceed 180° C.

A thermionic tube according to the invention contains at least one secondary-emission electrode a part of whose surface contains caesium oxide as an active secondary-emission material, the other non-activated parts of the surface of the electrode or electrodes being covered with the product obtained by reduction of one or more of the oxides of nickel, tungsten, zirconium or molybdenum.

The reduction of these metal oxides has the effect of producing on the secondary-emission electrode a layer consisting of the metal having such structure as to exhibit a black appearance. This metal may still be mixed with a quantity of metal oxide, since the reduction is effected only partly.

According to a process which also forms part 20 of the invention, a secondary-emission electrode is manufactured by applying, prior to its incorporation in the tube, to a part of the surface a layer consisting of one or more of the oxides of the metals nickel, tungsten, zirconium or molybdenum, and subsequently reducing this layer at low temperature.

The application of the metal oxides to the electrode may be effected, for example, by spraying, dipping, or with the aid of the cataphoretic 30 process.

The reduction at low temperature has the effect of producing a non-hardened, finely distributed structure of the metal which is particularly adapted to the emission of heat and the adherence 35 of small quantities of caesium.

According to one particular example of a process according to the invention, the reduction is effected during about 10 minutes at a temperature of about 700° C. The reduction may 40 take place, for example, in a hydrogen atmosphere.

We claim:

1. A secondary-emissive electrode for a thermionic tube having a multiplicity of parts on its 45 surface comprised of black particles of nickel, and secondary-emissive material on the said electrode around said nickel particles.

2. The process of making a secondary-emission electrode for a thermionic tube which comprises depositing nickel oxide on the surface of

2

said electrode, reducing said oxide to a metal in a hydrogen atmosphere at a temperature of about 700° C., and depositing secondary emissive material around said metal particles.

HENRI BIENFAIT.  
CORNELIS FREDERIK VEENEMANS.

## REFERENCES CITED

The following references are of record in the 10 file of this patent:

## UNITED STATES PATENTS

| Number    | Name                  | Date          |
|-----------|-----------------------|---------------|
| 2,123,024 | Piore et al. -----    | July 5, 1933  |
| 2,146,099 | De Boer et al. -----  | Feb. 7, 1939  |
| 2,171,227 | Schreinemachers --    | Aug. 29, 1939 |
| 2,190,695 | Bruining et al. ----- | Feb. 20, 1940 |
| 2,198,329 | Bruining et al. ----- | Apr. 23, 1940 |
| 2,204,252 | Krenzien -----        | June 11, 1940 |